

# UNITED STATES PATENT OFFICE.

FRED C. T. DANIELS, OF NATICK, MASSACHUSETTS.

## IRON ALLOY.

1,211,826.

Specification of Letters Patent.

Patented Jan. 9, 1917.

No Drawing.

Application filed April 3, 1916. Serial No. 88,718.

*To all whom it may concern:*

Be it known that I, FRED C. T. DANIELS, a citizen of the United States of America, residing at Natick, in the county of Middlesex 5 and State of Massachusetts, United States of America, have invented certain new and useful Improvements in Iron Alloys; and I do hereby declare the following to be a full, clear, and exact description of the invention, 10 such as will enable others skilled in the art to which it appertains to make and use the same.

My invention relates to a casting alloy of iron for casting sand rolls and like machinery parts for shaping hot or cold metal. It is especially adapted for rolls that take the place of chilled rolls for rolling mills, especially where on account of the width of the flanges of the shapes to be rolled, a deeply 20 chilled roll is necessary. Such a chilled roll is very difficult to make in the foundry, and is equally unsatisfactory to use in the rolling mill. For these reasons rolls of special iron alloys have recently been substituted for the 25 chilled rolls.

My alloy is used for the manufacture of rolls for rolling hot and cold iron and steel, forging and bending dies, rolling mill guides, pipe balls, shear knife edges and cutting tools, and for other high duty devices 30 and machines in which hardness combined with toughness and ability to resist wear and shocks to a high degree are most desirable and advantageous.

The object of my invention is to produce 35 a metal or alloy that is superior to other iron alloys and casting metals.

My new alloy is distinguished from known casting metals by a hardness exceeding 40 chilled iron rolls and also exceeding that of rolls of special alloys; by a decided toughness when heat treated, which almost coincides with that of manganese steel, and my metal differs therefrom not only in composition 45 and in the treatment thereof, but also in the uses to which it may be put, in that it may be cast into pieces of very large section, due to the fact that it does not require the same strenuous and sudden quenching and 50 annealing heat treatment that is required by manganese steel to produce its properties.

My alloy has the peculiar property, which I have never before encountered, that when

heated to 750° C., more or less, and maintained at that temperature for a length of 55 time, depending upon the thickness of the casting, of from one to sixty hours, and allowed to slowly cool, its hardness increases.

In addition to iron my alloy contains carbon, silicon, nickel and manganese, also other 60 elements usually present in iron alloys and kept within the usual limits of foundry practice, such as sulfur and phosphorus.

I am aware that iron alloys have been made containing these elements, but the proportions in which they are present are different from those in my alloy, and the properties of the alloys are not the same.

My alloy is essentially a high carbon casting iron containing nickel in large quantities 70 sufficient to impart the necessary hardness and toughness, and to which may be added more than the usual amount of manganese or silicon, or both manganese and silicon customary in foundry practice. 75

The nickel content ranges from about 1.00 per cent. to about 3.50 per cent. Such an alloy containing also silicon, phosphorus, sulfur and manganese (or any combination of these last elements within the usual foundry 80 practice ranges) gives a new and valuable alloy of iron. It is a white iron entirely throughout the casting, and is improved by heat treatment. Castings of this alloy are subjected to a prolonged heating by placing 85 them in a furnace and heating them from 700° to 850° C. for from one to sixty hours.

The length of time that the heating is continued is entirely dependent upon the thickness of the casting, it being my object to 90 heat the casting through and through to the temperatures above mentioned and then allow it to slowly cool. This can be done by closing the flues of the furnace and allowing the casting to remain therein until the temperature has dropped to about 125° C. to 95 250° C., when the casting may be taken out and allowed to cool in the open. This heat treatment not only removes the casting strains, but also greatly increases the toughness 100 of the alloy, which is a very valuable property of this alloy.

My invention also embraces the use of manganese in quantities in excess of the usual foundry practice, that is to say when 105 present in a high nickel high carbon iron in

quantities above one per cent., and suitably in quantities varying from one per cent. to the neighborhood of three per cent., has the important properties of hardening the metal 5 and improving its wearing surface, especially for rolls for rolling hot metal and which are plentifully supplied with cooling water.

My experience with casting irons shows 10 that the presence of manganese in the iron up to about .30 per cent. has a softening effect, that if the manganese content be increased from about .30 per cent. to about 1.00 per cent. known foundry practice, it 15 will have no noticeable effect on the high carbon iron, and that when the manganese content is increased over 1.00 per cent. and up to 2.75 per cent., it will have a strong hardening effect on the iron, have a tendency 20 to hold the carbon in the combined state, and will produce a better wearing surface in rolls well cooled by water.

My invention also consists in adding silicon in excess of the quantities used in general foundry practice to the high nickel high carbon iron, either with or without manganese, but always in such quantities that the resulting compound shall be a white iron.

30 My experience shows that when silicon is added to the mixture, whether manganese is present or not, the higher carbon limit above given cannot be used, and that the carbon content must be nearer the lower carbon limit above given, and specifically the carbon content of a high silicon iron cannot be much above 1.80 per cent. carbon in the absence of a high per cent. of manganese. When a high per cent. of manganese is present, however, a high percentage of silicon may be used with a much higher carbon content, namely 2.20 per cent. carbon and thereabout.

To the best of my knowledge silicon has 45 not been used in sand casting white irons in quantities over one per cent. and where the carbon range is over 1.25 per cent.

In my alloy the silicon may vary from 1.50 per cent. to 5.00 per cent. and imparts 50 to the alloy extreme hardness, especially in the presence of a high percentage of manganese and the upper permissible limits of carbon. Silicon is prone to convert the carbon into its graphitic state thereby producing a gray or black iron useless for the high duty purposes for which my alloy is made, and therefore care should be taken to control the proportion of the ingredients so as to produce a white iron.

60 The high percentage of silicon in the presence of the high percentage of manganese will produce a much harder and a much longer-wearing surface than when the manganese is not present, with the accompanying necessary lower carbon content.

Rolls of my new composition show a much longer wear, or, in other words, will produce more tonnage of rolled material for an equal amount of dressing than chilled rolls or rolls of other special iron alloys.

70

With the carbon over 2.20 per cent. the silicon should be kept under .75 per cent.; and while such a ratio of silicon to carbon has been known in other casting irons, they have not had the high nickel content of my 75 alloy, and consequently have not had the hardness, nor have they had the toughness, imparted to them by heat treatment.

The alloys of the compositions embraced in my invention are all white metal, and have exceptional properties; they have a tensile strength when not heat treated from 50,000 lbs. to 60,000 lbs. per square inch; when annealed as described, the tensile strength is increased from 75,000 lbs. per 85 square inch to 100,000 lbs. per sq. in., and this tensile strength is still further increased when forged hot.

The forgeability of the alloy after being heat treated when brought up to forging heat is an unexpected property, and is greater when the carbon content is low and when the silicon is present in the smaller quantities. For example, a high nickel low carbon iron with the silicon and other customary elements present within the ranges of ordinary foundry practice gave the following tests; cast material 60,000 lbs., annealed 100,000 lbs. forged hot, 140,000 lbs. per sq. in. The tensile strength of other forged compositions made in accordance with my invention with and without either or both silicon and manganese varied between this high limit of 140,000 lbs. per sq. in., to 100,000 lbs. per sq. in. The raw, that 95 is the unheat-treated metal, the heat-treated metal and the forged metal, when cold show no noticeable elongation in the testing machine. Their hardness as tested by the scleroscope or sclerometer is shown to be 100 above that of any iron alloys with which I am acquainted. The hardness of my raw material as so measured ranges from 55 to 70; of the toughened heat-treated material 105 from 60 to 85 and the forged material 110 115 for the various compositions.

Manganese is preferably present in all the compositions in quantity sufficient to impart fluidity and soundness to the material.

Another peculiarity is that the presence 120 of small quantities of vanadium, tungsten, copper, molybdenum, aluminum, chromium, cobalt, and titanium and similar elements, have given no noticeable alteration in the properties of my alloy, whether present in the original ore, pig or scrap, or added as elements, alloys or ferro-alloys. Specimens of alloys made in accordance with my invention were found to be non-magnetic when cast; magnetic after heat treatment as above 125 130 135

described, and when quenched loses its magnetic properties.

Examples of white irons which I have made are represented by the following 5 analyses:

|    | Si.      | S.       | P.       | Mn.       | C.        | Ni.       |         |
|----|----------|----------|----------|-----------|-----------|-----------|---------|
| 10 | .40-1.50 | .01-.20  | .01-1.50 | .01-1.00  | 1.25-2.20 | 1.00-3.50 |         |
|    | .20-85   | ...do... | ...do... | ...do...  | 2.20-3.50 | ...do...  | Iron to |
|    | .40-1.25 | ...do... | ...do... | 1.00-3.75 | 1.25-2.20 | ...do...  | make    |
|    | .20-85   | ...do... | ...do... | ...do...  | 2.20-3.50 | ...do...  | 100%.   |
|    | 1.50-500 | ...do... | ...do... | 10-1.00   | .89-1.80  | ...do...  |         |
|    | ...do... | ...do... | ...do... | 1.00-2.75 | .89-2.20  | ...do...  |         |

A few specific analyses of individual heats 15 are given by way of example, as follows:

|    | Si.    | S.   | P.    | Mn.   | C.    | Ni.  |      |
|----|--------|------|-------|-------|-------|------|------|
| 20 | a..... | 0.73 | 0.028 | 0.033 | 0.260 | 1.76 | 3.14 |
|    | b..... | 0.60 | 0.050 | 0.040 | 0.300 | 2.80 | 1.76 |
|    | c..... | 0.42 | 0.088 | 0.220 | 2.260 | 3.06 | 2.12 |
|    | d..... | 0.88 | 0.030 | 0.043 | 1.760 | 1.90 | 2.20 |
|    | e..... | 2.00 | 0.041 | 0.040 | 0.280 | 1.76 | 2.22 |
|    | f..... | 3.30 | 0.036 | 0.036 | 1.800 | 1.87 | 2.45 |

The color of the raw alloy is like that of 25 cast steel, and the color when heat-treated is like that of annealed steel. The fracture of the raw product (un-heat-treated) is bright crystalline, the fracture of the heat-treated product is dull. The dressed surface of the 30 raw product is bright and shiny, that of the heat-treated product is dull and silky.

It is, of course, well understood that it is difficult to obtain different large molten masses of iron alloy having exactly the same 35 composition, and slight variations in the proportions of the ingredients comprising my alloy shall be deemed within the terms of my invention.

The alloy should be run into the molds at 40 a casting temperature between 1200° C. and 1350° C., and preferably between 1225° C. and 1235° C.

My alloy is hard, long-wearing, tough, and shock-resisting, exhibiting all of these 45 properties to a greater extent than any other iron alloy with which I am acquainted.

I claim—

1. An iron alloy containing silicon, sulfur, phosphorus, manganese, combined carbon from 1.25% to 3.50%, and nickel from 50 1.00% to 3.50%, the relative proportions of

the said elements being maintained to produce a white iron under all conditions.

2. An iron alloy containing silicon, sulfur, phosphorus, combined carbon from 55 1.25% to 3.50%, nickel from 1.00% to 3.50%, and a manganese content above the percentage used in foundry irons, the relative proportions of said elements being maintained to produce a white iron.

3. An iron alloy containing silicon, sulfur, phosphorus, combined carbon from 60 1.25% to 3.50%, nickel from 1.00% to 3.50%, manganese from 1.00% to 2.75%, the relative proportions of said elements being maintained to produce a white iron.

4. A white casting metal, an alloy of iron containing sulfur, phosphorus and manganese, and also containing carbon from 65 1.25% to 2.20% in the presence of a nickel content from 1.00% to 3.50% and silicon from 1.00% to 5.00%.

5. A white casting metal, an iron alloy containing sulfur and phosphorus, and also 70 containing carbon from 1.25% to 2.20%, nickel from 1.00% to 3.50%, manganese from 1.00% to 2.75%, and silicon from 1.00% to 5.00%.

6. A white casting metal, an alloy of iron containing sulfur and phosphorus, and also 75 containing carbon from 1.25% to 2.20% in the presence of nickel from 1.00% to 3.50% and a high manganese and a high silicon content.

7. A white casting metal, an alloy of iron containing sulfur and phosphorus and also 80 containing carbon from 1.25% to 2.20% in the presence of a nickel content of 1.00% to 3.50% and a high silicon content commensurate with respect to the carbon content.

8. A white casting metal, an alloy of iron, containing manganese about .73% silicon, about .028% sulfur, about .033% phosphorus, about 1.76% carbon and about 85 3.14% nickel.

In testimony that I claim the foregoing as my invention, I have signed my name in presence of two subscribing witnesses.

FRED C. T. DANIELS.

Witnesses:

H. J. SCHURFLER,

A. E. SCHUBART.